

# UNITED STATES PATENT OFFICE.

GEORGE D. VAN ARSDALE, OF EAST ORANGE, NEW JERSEY.

## PROCESS FOR ELECTROLYTICALLY REFINING COPPER.

1,069,305.

Specification of Letters Patent.

Patented Aug. 5, 1913.

No Drawing.

Application filed October 2, 1908. Serial No. 455,826.

*To all whom it may concern:*

Be it known that I, GEORGE D. VAN ARSDALE, a citizen of the United States of America, and a resident of East Orange, county of Essex, and State of New Jersey, have invented a certain new and Improved Process for Electrolytically Refining Copper, of which the following is a specification.

10 In the electrolytic refining of copper, as practised at the present day, the electrolyte employed is usually an acid solution of copper sulfate in which the copper present is in the cupric state. The employment of a 15 cuprous compound in this connection, such as would fulfil the requirements of an electrolytic process, would be much more economical because a very much less power,—theoretically exactly one-half of the amount 20 needed when cupric compounds are employed,—is necessary when the copper is contained in a cuprous state. Many cuprous compounds however, are not soluble or are but slightly soluble and hence are 25 not available. Furthermore, a number of soluble cuprous compounds are readily oxidizable and hence though cuprous when first employed would quickly pass to the cupric form. And again, certain cuprous compounds which might otherwise be available 30 for this purpose, are useless on account of their action on certain constituents of the copper to be purified. I have found, however, by experiment, that solutions of certain cuprous compounds form suitable electrolytes for electrolytically refining copper, and when thus employed result in the deposition of substantially double the amount of metal in a given time, and with a given ex- 35 penditure of power, which would be deposited in an apparatus employing electrolytes comprising solutions of cupric salts. For example: There are several sulfites of copper and a number of double salts of the 40 same which when in solution form suitable electrolytes. A solution of cupric sulfate may be made strongly ammoniacal and then impregnated with sulfur dioxide gas until all the copper is reduced to the cuprous 45 state. The copper will then be probably in the form of the double salt, ammonium cuprous sulfite, which will be kept in solution by other salts present. As another ex-

ample,—a readily soluble sulfite, such as sodium or ammonium sulfite, may be added 55 in excess to a solution of a cupric salt; or any cuprous sulfite, already existing as such, may be dissolved by the addition of certain salts, such as sodium or ammonium or other readily soluble sulfites; or such reducing agents as phosphorous acid or phosphites may be used in a similar manner.

In carrying out the process of purifying and refining the copper, I employ the copper to be treated as the anode in an electrolytic apparatus containing the above defined electrolyte, and provide a suitable cathode for receiving the deposit. I then pass a current of electricity through the bath whereby copper is dissolved from the anode, 65 passes through the electrolyte and is deposited upon the cathode in a refined and pure condition. The impurities are received or retained in the electrolyte and are then in a form convenient for further treatment, 70 but in the meantime the solution remains of uniform strength so far as copper is concerned, because substantially no more copper will be deposited upon the cathode than is dissolved from the anode.

80 Other salts or substances may be added to the electrolytic solution for specific purposes, as may be desired, such as for increasing the conductivity thereof, or for decreasing the tendency to polarization, and 85 details as to strength of solution, temperature, etc., may be varied to suit varying conditions.

The purification of the solution from accumulated impurities, may be carried out in 90 any desired manner, as this part of the process forms no part of my present invention.

What I claim is:

1. The herein described process of refining metallic copper which consists in dissolving the same electrolytically from a metallic anode thereof immersed in an electrolyte containing a soluble cuprous sulfite, and depositing the dissolved copper 100 upon a cathode also immersed within the said electrolyte.

2. The herein described process of refining metallic copper which consists in dissolving the same electrolytically from a metallic anode thereof immersed in an elec- 105

troyte containing ammonium cuprous sulfite, and depositing the dissolved copper upon a cathode also immersed within the said electrolyte.

- 5 3. The herein described process which consists in separating copper by electrolysis from an electrolyte containing copper in

the cuprous state, the electrolyte also containing a soluble sulfite.

GEORGE D. VAN ARSDALE.

Witnesses:

D. HOWARD HAYWOOD,  
LYMAN S. ANDREWS, Jr.